



US009327519B1

(12) **United States Patent**  
**Larson et al.**

(10) **Patent No.:** **US 9,327,519 B1**  
(45) **Date of Patent:** **May 3, 2016**

(54) **SACRIFICIAL COATING AND INDIRECT PRINTING APPARATUS EMPLOYING SACRIFICIAL COATING ON INTERMEDIATE TRANSFER MEMBER**

(71) Applicant: **XEROX CORPORATION**, Norwalk, CT (US)

(72) Inventors: **James R. Larson**, Fairport, NY (US); **Jeffrey J. Folkins**, Rochester, NY (US); **Santokh S. Badesha**, Pittsford, NY (US); **Mandakini Kanungo**, Penfield, NY (US)

(73) Assignee: **XEROX CORPORATION**, Norwalk, CT (US)

(\*) Notice: Subject to any disclaimer, the term of this patent is extended or adjusted under 35 U.S.C. 154(b) by 0 days.

(21) Appl. No.: **14/867,864**

(22) Filed: **Sep. 28, 2015**

(51) **Int. Cl.**  
**B41J 11/00** (2006.01)

(52) **U.S. Cl.**  
CPC ..... **B41J 11/0015** (2013.01)  
(58) **Field of Classification Search**  
CPC .. B41J 11/0015; B41J 2002/012; B41J 2/005;  
B41J 2/0057; B41J 2/01; B41M 5/50  
See application file for complete search history.

(56) **References Cited**

U.S. PATENT DOCUMENTS

2003/0067528 A1\* 4/2003 Chowdry et al. .... B41J 2/04  
347/103



OTHER PUBLICATIONS

Song et al., "Sacrificial Coating and Indirect Printing Apparatus Employing Sacrificial Coating on Intermediate Transfer Member," U.S. Appl. No. 14/665,319, filed Mar. 23, 2015.

Larson et al., "Sacrificial Coating and Indirect Printing Apparatus Employing Sacrificial Coating on Intermediate Transfer Member," U.S. Appl. No. 14/830,557, filed Aug. 19, 2015.

\* cited by examiner

*Primary Examiner* — Thinh Nguyen

(74) *Attorney, Agent, or Firm* — MH2 Technology Law Group LLP

(57) **ABSTRACT**

An indirect printing process comprises providing an inkjet printing apparatus comprising an intermediate transfer member. A wet sacrificial coating composition is deposited onto the intermediate transfer member. The wet sacrificial coating composition is made from ingredients comprising: a waxy starch; at least one hygroscopic material; at least one surfactant; and a liquid carrier. The wet sacrificial coating composition is dried to form a dry sacrificial coating. Droplets of ink are ejected in an imagewise pattern onto the dry sacrificial coating. The ink is at least partially dried to form a substantially dry ink pattern. Both the substantially dry ink pattern and the sacrificial coating are transferred from the intermediate transfer member to a final substrate. At least one cross-linking agent is applied to cross-link the sacrificial coating. The cross-linking agent is applied to at least one of: a) the intermediate transfer member prior to depositing the wet sacrificial coating composition, b) the wet sacrificial coating composition after depositing the wet sacrificial coating composition onto the intermediate transfer member, c) the dry sacrificial coating on the intermediate transfer member, d) the dry sacrificial coating on the final substrate.

**20 Claims, 10 Drawing Sheets**





FIG. 2



FIG. 3



FIG. 4A



FIG. 4B



FIG. 4C



FIG. 4D



FIG. 4E



FIG. 5A



FIG. 5B

## WATER FASTNESS RESULTS - PACIFIC FIXTURE - BLACK

% RATIO IN OD: PACIFIC PRINTS - BLACK



FIG. 6

## WATER FASTNESS RESULTS - PACIFIC FIXTURE - MAGENTA

% RATIO IN OD: PACIFIC PRINTS - MAGENTA



FIG. 7



FIG. 8



FIG. 9



FIG. 10A



FIG. 10B

**SACRIFICIAL COATING AND INDIRECT  
PRINTING APPARATUS EMPLOYING  
SACRIFICIAL COATING ON INTERMEDIATE  
TRANSFER MEMBER**

Identifying and developing new polymer coating materials that provide good wet image quality and/or image transfer with improved water fastness would be considered a welcome advance in the art.

5

**FIELD OF THE DISCLOSURE**

This disclosure relates generally to indirect inkjet printers, and in particular, to a sacrificial coating employed on an intermediate transfer member of an inkjet printer.

**BACKGROUND**

In aqueous ink indirect printing, an aqueous ink is jetted on to an intermediate imaging surface, which can be in the form of a blanket. The ink is partially dried on the blanket prior to transfixing the image to a media substrate, such as a sheet of paper. To ensure excellent print quality it is desirable that the ink drops jetted onto the blanket spread and become well-coalesced prior to drying. Otherwise, the ink images appear grainy and have deletions. Lack of spreading can also cause failing inkjet ejectors to be much more apparent, producing broader streaks in the ink image. Spreading of aqueous ink is facilitated by materials having a high surface energy.

However, in order to facilitate transfer of the ink image from the blanket to the media substrate after the ink is dried on the intermediate imaging surface, a blanket having a surface with a relatively low surface energy is preferred. Rather than providing the desired spreading of ink, low surface energy materials tend to promote “beading” of individual ink drops on the image receiving surface.

Thus, an optimum blanket for an indirect image transfer process must tackle both the challenges of wet image quality, including desired spreading and coalescing of the wet ink; and the image transfer of the dried ink. The first challenge—wet image quality—prefers a high surface energy blanket that causes the aqueous ink to spread and wet the surface. The second challenge—image transfer—prefers a low surface energy blanket so that the ink, once partially dried, has minimal attraction to the blanket surface and can be transferred to the media substrate.

Various approaches have been investigated to provide a solution that balances the above challenges. These approaches include blanket material selection, ink design and auxiliary fluid methods. With respect to material selection, materials that are known to provide optimum release properties include the classes of silicone, fluorosilicone, a fluoropolymer, such as TEFLO or VITON, and certain hybrid materials. These materials have low surface energy, but provide poor wetting. Alternatively, polyurethane and polyimide have been used to improve wetting, but at the cost of ink release properties. Tuning ink compositions to address these challenges has proven to be very difficult since the primary performance attribute of the ink is the performance in the print head. For instance, if the ink surface tension is too high it may not jet properly, depending on type of printheads, and if it is too low it may drool out of the face plate of the printhead.

In addition to affecting image quality and transfer characteristics of the ink, the sacrificial coating properties can also affect water fastness of the prints. Water fastness is a known concern for aqueous inks generally. Poor water fastness can result in smudging, reduced image quality and unwanted transfer of ink such as to the fingers of users handling the images.

5

**SUMMARY**

An embodiment of the present disclosure is directed to an indirect printing process. The process comprises providing an inkjet printing apparatus comprising an intermediate transfer member. A wet sacrificial coating composition is deposited onto the intermediate transfer member. The wet sacrificial coating composition is made from ingredients comprising: a waxy starch; at least one hygroscopic material; at least one surfactant; and a liquid carrier. The wet sacrificial coating composition is dried to form a dry sacrificial coating. Droplets of ink are ejected in an imagewise pattern onto the dry sacrificial coating. The ink is at least partially dried to form a substantially dry ink pattern. Both the substantially dry ink pattern and the sacrificial coating are transferred from the intermediate transfer member to a final substrate. At least one cross-linking agent is applied to cross-link the sacrificial coating. The cross-linking agent is applied to at least one of: a) the intermediate transfer member prior to depositing the wet sacrificial coating composition, b) the wet sacrificial coating composition after depositing the wet sacrificial coating composition onto the intermediate transfer member, c) the dry sacrificial coating on the intermediate transfer member, d) the dry sacrificial coating on the final substrate.

The sacrificial coating compositions of the present disclosure can provide one or more of the following advantages: coatings having good wettability, coatings having good ink wetting and ink spreading, image transfer member coatings exhibiting improved wet image quality and/or improved image transfer with aqueous inks, improved physical robustness or increased shelf life, improved image quality; or improved water fastness.

It is to be understood that both the foregoing general description and the following detailed description are exemplary and explanatory only and are not restrictive of the present teachings, as claimed.

**BRIEF DESCRIPTION OF THE DRAWINGS**

The accompanying drawings, which are incorporated in and constitute a part of this specification, illustrate embodiments of the present teachings and together with the description, serve to explain the principles of the present teachings.

FIG. 1 is a schematic drawing of an aqueous indirect inkjet printer that prints sheet media, according to an embodiment of the present disclosure.

FIG. 2 is a schematic drawing of a surface maintenance unit that applies a hydrophilic sacrificial coating composition to a surface of an intermediate transfer member in an inkjet printer, according to an embodiment of the present disclosure.

FIG. 3 is a block diagram of a process for printing images with an indirect inkjet printer that uses aqueous inks, according to an embodiment of the present disclosure.

FIG. 4A is a side view of a hydrophilic sacrificial coating composition that is formed on the surface of an intermediate transfer member in an inkjet printer, according to an embodiment of the present disclosure.

FIG. 4B is a side view of dried or semi-dried hydrophilic sacrificial coating composition on the surface of the intermediate transfer member after a dryer removes a portion of a liquid carrier in the hydrophilic sacrificial coating composition, according to an embodiment of the present disclosure.

FIG. 4C is a side view of a portion of an aqueous ink image that is formed on the dried or semi-dried hydrophilic sacrificial coating composition on the surface of the intermediate transfer member, according to an embodiment of the present disclosure.

FIG. 4D is a side view of a portion of the aqueous ink image that is formed on the dried hydrophilic sacrificial coating composition after a dryer in the printer removes a portion of the water in the aqueous ink, according to an embodiment of the present disclosure.

FIG. 4E is a side view of a print medium that receives the aqueous ink image and a portion of the dried layer of the hydrophilic sacrificial coating composition after a transfix operation in the inkjet printer, according to an embodiment of the present disclosure.

FIG. 5A shows a graph of water fastness data for airbrush test samples, according to examples of the present disclosure.

FIG. 5B shows visual results of water fastness testing for airbrush test samples, according to examples of the present disclosure.

FIG. 6 shows a graph of smear ratio testing for black ink, according to examples of the present disclosure.

FIG. 7 shows a graph of smear ratio testing for magenta ink, according to examples of the present disclosure.

FIG. 8 shows a graph of smear ratio testing for black ink, according to examples of the present disclosure.

FIG. 9 shows a graph of smear ratio testing for magenta ink, according to examples of the present disclosure.

FIGS. 10A and 10B show water fastness screening test results for an ink:skin ratio of 25:75, according to examples of the present disclosure.

It should be noted that some details of the figure have been simplified and are drawn to facilitate understanding of the embodiments rather than to maintain strict structural accuracy, detail, and scale.

#### DESCRIPTION OF THE EMBODIMENTS

Reference will now be made in detail to embodiments of the present teachings, examples of which are illustrated in the accompanying drawings. In the drawings, like reference numerals have been used throughout to designate identical elements. In the following description, reference is made to the accompanying drawing that forms a part thereof, and in which is shown by way of illustration a specific exemplary embodiment in which the present teachings may be practiced. The following description is, therefore, merely exemplary.

As used herein, the terms “printer,” “printing device,” or “imaging device” generally refer to a device that produces an image on print media with aqueous ink and may encompass any such apparatus, such as a digital copier, bookmaking machine, facsimile machine, multi-function machine, or the like, which generates printed images for any purpose. Image data generally include information in electronic form which are rendered and used to operate the inkjet ejectors to form an ink image on the print media. These data can include text, graphics, pictures, and the like. The operation of producing images with colorants on print media, for example, graphics, text, photographs, and the like, is generally referred to herein as printing or marking. Aqueous inkjet printers use inks that have a high percentage of water relative to the amount of colorant and/or solvent in the ink.

The term “printhead” as used herein refers to a component in the printer that is configured with inkjet ejectors to eject ink drops onto an image receiving surface. A typical printhead includes a plurality of inkjet ejectors that eject ink drops of one or more ink colors onto the image receiving surface in

response to firing signals that operate actuators in the inkjet ejectors. The inkjets are arranged in an array of one or more rows and columns. In some embodiments, the inkjets are arranged in staggered diagonal rows across a face of the printhead. Various printer embodiments include one or more printheads that form ink images on an image receiving surface. Some printer embodiments include a plurality of printheads arranged in a print zone. An image receiving surface, such as an intermediate imaging surface, moves past the printheads in a process direction through the print zone. The inkjets in the printheads eject ink drops in rows in a cross-process direction, which is perpendicular to the process direction across the image receiving surface.

As used in this document, the term “aqueous ink” includes liquid inks in which colorant is in a solution, suspension or dispersion with a liquid vehicle that includes water and/or one or more liquid solvents. The terms “liquid solvent” or more simply “solvent” are used broadly to include compounds that may dissolve colorants into a solution, or that may be a liquid that holds particles of colorant in a suspension or dispersion without dissolving the colorant.

As used herein, the term “hydrophilic” refers to any composition or compound that attracts water molecules or other solvents used in aqueous ink. As used herein, a reference to a hydrophilic composition refers to a liquid carrier that carries a hydrophilic agent. Examples of liquid carriers include, but are not limited to, a liquid, such as water or alcohol, that carries a dispersion, suspension, or solution.

As used herein, a reference to a dried layer or dried coating refers to an arrangement of a hydrophilic compound after all or a substantial portion of the liquid carrier has been removed from the composition through a drying process. As described in more detail below, an indirect inkjet printer forms a layer of a hydrophilic composition on a surface of an intermediate transfer member using a liquid carrier, such as water, to apply a layer of the hydrophilic composition to an image receiving surface to form a uniform layer of the hydrophilic composition on the image receiving surface.

An embodiment of the present disclosure is directed to an indirect printing process. The process comprises providing an inkjet printing apparatus comprising an intermediate transfer member. A wet sacrificial coating composition is deposited onto the intermediate transfer member. The wet sacrificial coating composition is made from ingredients comprising: a waxy starch; at least one hygroscopic material; at least one surfactant; and a liquid carrier. The wet sacrificial coating composition is dried to form a dry sacrificial coating. Droplets of ink are ejected in an imagewise pattern onto the dry sacrificial coating. The ink is at least partially dried to form a substantially dry ink pattern. Both the substantially dry ink pattern and the sacrificial coating are transferred from the intermediate transfer member to a final substrate, also referred to herein as a print medium. As part of the process, at least one cross-linking agent is applied to cross-link the sacrificial coating. The cross-linking agent is applied to at least one of: a) the intermediate transfer member prior to depositing the wet sacrificial coating, b) the wet sacrificial coating composition after depositing the wet sacrificial coating composition onto the intermediate transfer member, c) the dry sacrificial coating on the intermediate transfer member, and d) the dry sacrificial coating on the final substrate.

The cross-linking agents of the present disclosure are not pre-mixed with the sacrificial coating compositions of the present disclosure. Premixing of the cross-linking agents can potentially cause premature cross-linking of the composition, which may result in instability of the coating solutions (e.g.,

precipitation of the starch and/or other coating precursors from solution prior to deposition of the sacrificial coating). The processes of the present disclosure can solve the problem of potential premature cross-linking by bringing the cross-linking agent into contact with the sacrificial coating compositions after or simultaneously with deposition of the coating compositions. Employing a cross linking agent or agents as part of a sacrificial coating composition on an intermediate transfer member of an aqueous inkjet printer is described in related U.S. application Ser. No. 14/665,319, filed Mar. 23, 2015, and U.S. application Ser. No. 14/830,557, filed Aug. 19, 2015, the disclosures of both of which applications are incorporated herein by reference in their entireties.

As mentioned above, the sacrificial coating composition employed in the process of the present disclosure comprises a waxy starch. In an embodiment, the waxy starch is a waxy maize starch. For example, the waxy maize starch can be a cationic waxy maize starch or a non-cationic waxy maize starch. Examples of cationic starch include acid treated waxy maize starch, as described for example, in U.S. patent application Ser. No. 14/219,125, filed Mar. 19, 2014, in the name of Guiqin Song et al., and entitled "WETTING ENHANCEMENT COATING ON INTERMEDIATE TRANSFER MEMBER (ITM) FOR AQUEOUS INKJET INTERMEDIATE TRANSFER ARCHITECTURE," the disclosure of which is incorporated herein by reference in its entirety. Suitable non-cationic waxy maize starches include acid depolymerized waxy starch, available from Cargill, Inc. as CALIBER® 180. The waxy starch may also be any other kind of waxy starch other than a waxy maize starch, such as a waxy rice starch, a waxy cassava starch, a waxy potato starch, a waxy wheat starch and a waxy barley starch. The viscosity of the at least one waxy starch, such as waxy maize starch, at about 25° C. may be less than about 1000 cps at a starch solid content of about 4%, such as less than about 700 cps, or less than 500 cps.

In certain embodiments disclosed herein, the at least one waxy starch may be gelatinized. Starch gelatinization is a process that breaks down the intermolecular bonds of starch molecules in the presence of water and heat, allowing the hydrogen bonding sites (the hydroxyl hydrogen and oxygen) to engage more water. Therefore heating the at least one waxy starch in the presence of water irreversibly dissolves the starch granule. For example, a waxy starch slurry can be prepared by mixing deionized water with a desired amount of starch, such as a solid starch content of from about 1 weight percent to about 30 weight percent, based on the total weight of the slurry. The starch slurry is gelatinized, or cooked out, either in a batch process or by a jet cooker. For batch process, the starch slurry can be heated to a temperature of, for example, from about 93° C. to about 98° C., and kept at this temperature for about 15 minutes to about 60 minutes.

The waxy starch can be used in any suitable amount. In an embodiment, the weight percent of the starch in the wet sacrificial coating of the present disclosure ranges from about 0.5 weight percent to about 10 weight percent, such as about 1 to about 8, or about 2 to about 6 weight percent, based on the total weight of the wet sacrificial coating composition.

Polyvinyl alcohol (PVOH) and copolymers thereof are optionally included with the starch as part of the binder in the sacrificial coating compositions of the present disclosure. In an embodiment, the waxy starch and the at least one PVOH and/or PVOH co-polymer are respectively in a weight ratio ranging from about 2:1 to about 20:1, such as about 3:1 to about 16:1, or about 4:1.

The PVOH and copolymers thereof can be selected from the group consisting of i) polyvinyl alcohol and ii) a copoly-

mer of vinyl alcohol and alkene monomers. In an embodiment, the at least one polymer is polyvinyl alcohol. In an embodiment, the at least one polymer is a copolymer of polyvinyl alcohol and alkene monomers. Examples of suitable polyvinyl alcohol copolymers include poly(vinyl alcohol-co-ethylene). In an embodiment, the poly(vinyl alcohol-co-ethylene) has an ethylene content ranging from about 5 mole % to about 30 mole %. Other examples of polyvinyl copolymer include poly(acrylic acid)-poly(vinyl alcohol) copolymer, polyvinyl alcohol-acrylic acid-methyl methacrylate copolymer and poly(vinyl alcohol-co-aspartic acid) copolymer. One example of a commercially available PVOH is SELVOL™ PVOH 825, available from Sekisui Specialty Chemicals of Dallas, Tex.

It is well known that PVOH can be manufactured by hydrolysis of polyvinyl acetate from, for example, partially hydrolyzed (87-89%), intermediate hydrolyzed (91-95%), fully hydrolyzed (98-98.8%) to super hydrolyzed (more than 99.3%). In an embodiment, the polyvinyl alcohol employed in the compositions of the present disclosure has a hydrolysis degree of at least 95% or higher, or at least 98% or 99.3% or higher.

The polyvinyl alcohol or copolymer thereof can have any suitable molecular weight. In an embodiment, the weight average molecular weight ranges from about 85,000 to about 186,000, such as from about 90,000 to about 180,000, or from about 100,000 to about 170,000, or from about 120,000 to about 150,000. Employing relatively high molecular weight PVOH can generate a strong thin film when combined with the starch and help to transfer the film onto the blanket. The loading of the PVOH is not higher than 50%, since higher loading of high molecular weight PVOH can significantly increase the viscosity and result in coating problems.

In an embodiment, the polyvinyl alcohol can have a suitable viscosity for forming a sacrificial coating on an intermediate transfer member. For example, at about 4% by weight of the polyvinyl alcohol in a solution of deionized water, and at a temperature of 20° C., the viscosity can be at least 20 centipoises ("cps"), such as 25, 26 or 30 cps or higher, where the % by weight of polyvinyl alcohol is relative to the total weight of polyvinyl alcohol and water.

Polyvinyl alcohol is a hydrophilic polymer and has good water retention properties. As a hydrophilic polymer, the coating film formed from polyvinyl alcohol can also exhibit good water retention properties, which can assist the ink spreading on the blanket. Because of its superior strength, coatings formulated with polyvinyl alcohol may achieve a significant reduction in total solid loading level. This may provide substantial cost savings while providing a significant improvement of the coating film performance. Polyvinyl alcohol and starch based sacrificial coating compositions may have improved mechanical properties and provide improved printer run-ability compared to other known sacrificial coating compositions, such as, for example, improved ink skin transfer properties, particularly for long printing runs. Moreover, both polyvinyl alcohol and starch are considered environmentally friendly, an important characteristic when used in sacrificial coating compositions.

The chemical structure of the starch and optional polyvinyl alcohol containing coating can be tailored to fine-tune the wettability and release characteristics of the sacrificial coating from the underlying ITM surface. This can be accomplished by employing one or more hygroscopic materials and one or more surfactants in the coating composition. However, employing a starch-PVOH based sacrificial coating with hygroscopic materials can adversely affect the water fastness of inkjet prints. While the use of the hygroscopic materials in

combination with the starch binder may exacerbate problems with water fastness, the inventors have found that the use of the cross-linking agents described above can minimize and in many cases eliminate the problem.

Any suitable hygroscopic material can be employed in the sacrificial coating compositions of the present disclosure. Hygroscopic materials can include substances capable of absorbing water from their surroundings, such as humectants. In an embodiment, the hygroscopic material can be a compound that is also functionalized as a plasticizer. In an embodiment, the at least one hygroscopic material is selected from the group consisting of glycerol, sorbitol or glycols such as polyethylene glycol, and mixtures thereof. A single hygroscopic material can be used. Alternatively, multiple hygroscopic materials, such as two, three or more hygroscopic materials, can be used.

Any suitable surfactants can be employed. Examples of suitable surfactants include anionic surfactants, cationic surfactants, non-ionic surfactants and mixtures thereof. The non-ionic surfactants can have an HLB value ranging from about 4 to about 14. A single surfactant can be used. Alternatively, multiple surfactants, such as two, three or more surfactants, can be used. For example, the mixture of a low HLB non-ionic surfactant with a value from about 4 to about 8 and a high HLB non-ionic surfactant with value from about 10 to about 14 demonstrates good wetting performance. In an embodiment, the at least one surfactant is sodium lauryl sulfate ("SLS").

The wet compositions of the present disclosure include a liquid carrier. The liquid carrier can be an aqueous based carrier, such as a carrier comprising at least 50% by weight water, such as 90% or 95% by weight or more water, such as 100%. Other ingredients that can be included as part of the aqueous based carrier system include organic solvents, such as ketones. An example of a ketone solvent is 2-Pyrrolidinone, which can potentially replace some loading of the glycerol. Other organic solvents that can be used in addition to or in place of 2-Pyrrolidinone include terpineol; dimethylsulfoxide; N-methylpyrrolidone; 1,3-dimethyl-2-imidazolidinone; 1,3-dimethyl-3,4,5,6-tetrahydro-2-pyrimidinone; dimethylpropylene urea; isopropanol, MEK (methyl ethyl ketone) and mixtures thereof. The organic solvents can have benefits, such as to improve film forming property, control drying characteristics and control wetting property of the semi-dry sacrificial layer. In an embodiment, the aqueous based carrier is 100% water.

Initially, the sacrificial coating composition is applied to the intermediate transfer member ("ITM"), where it is semi-dried or dried to form a film. The coating can have a higher surface energy and/or be more hydrophilic than the base ITM, which is usually a material with low surface free energy, such as, for example, a polysiloxane, such as polydimethylsiloxane or other silicone rubber material, fluorosilicone, TEFLON, polyimide or combinations thereof.

In an embodiment, the sacrificial coating is made by mixing the ingredients comprising: a waxy starch; at least one hygroscopic material; at least one surfactant; a liquid carrier and optionally at least one polymer selected from the group consisting of i) polyvinyl alcohol and ii) a copolymer of vinyl alcohol and alkene monomers.

In addition to the ingredients discussed above, the mixture can include other ingredients, such as biocides. Example biocides include ACTICIDES® CT, ACTICIDES® LA 1209 and ACTICIDES® MBS in any suitable concentration, such as from about 0.1 weight percent to about 2 weight percent.

The ingredients of the sacrificial coating can be mixed in any suitable manner to form a composition that can be coated

onto the intermediate transfer member. The ingredients can be mixed in any suitable amounts. For example, the waxy starch can be added in an amount of from about 0.5 to about 10 weight percent, or from about 2 to about 8, or from about 5 to about 7 weight percent based upon the total weight of the coating mixture. The optional polyvinyl alcohol or vinyl alcohol copolymer can be added in an amount of from about 0 to about 5% by weight, or from about 0.5 to about 4% by weight, or from about 1 to about 3% by weight, based upon the total weight of the coating mixture. The surfactants can be present in an amount of from about 0.01 to about 4% by weight, or from about 0.05 to about 2% by weight, or from about 0.08 to about 1% by weight, based upon the total weight of the coating mixture. The hygroscopic material can be present in an amount of from about 0.5 to about 30% by weight, or from about 2 to about 25 by weight, or from about 4 to about 20% by weight, or about 10 to about 15% by weight, based upon the total weight of the coating mixture.

The compositions of the present disclosure can be used to form a sacrificial coating over any suitable substrate. Any suitable coating method can be employed, including, but not limited to, dip coating, spray coating, spin coating, flow coating, stamp printing, die extrusion coatings, flexo and gravure coating and/or blade techniques. In exemplary embodiments, suitable methods can be employed to coat the liquid sacrificial coating composition on an intermediate transfer member, such as, for example, use of an anilox roller, as shown in FIG. 2; or an air atomization device, such as an air brush or an automated air/liquid sprayer can be used for spray coating. In another example, a programmable dispenser can be used to apply the coating material to conduct a flow coating.

As described above, the sacrificial coating is first applied or disposed as a wet coating on the intermediate transfer member. A drying or curing process can then be employed. In embodiments, the wet coating can be heated at an appropriate temperature for the drying and curing, depending on the material or process used. For example, the wet coating can be heated to a temperature ranging from about 30° C. to about 200° C. for about 0.01 to about 100 seconds or from about 0.1 second to about 60 seconds. Also, the speed of air flow can be adjusted during the drying process to accelerate drying at low temperature. In embodiments, after the drying and curing process, the sacrificial coating can have a thickness ranging from about 0.02 micrometer to about 10 micrometers, or from about 0.02 micrometer to about 5 micrometers, or from about 0.05 micrometer to about 1 micrometers.

In an embodiment, the sacrificial coating can cover a portion of a major surface of the intermediate transfer member. The major outer surface of the intermediate transfer member can comprise, for example, polysiloxanes, fluoro-silicones, fluoropolymers such as VITON or TEFLON and the like.

It has been found that the sacrificial coating overcomes the wet image quality problem discussed above by providing an ink wetting surface on the intermediate transfer member. The coatings may also improve the image cohesion significantly to enable excellent image transfer.

The at least one cross-linking agent employed in the process of the present disclosure can be any compound that is suitable for cross-linking the waxy starch and optional polyvinyl alcohol and/or copolymers thereof in the sacrificial coating composition at a temperature and in a period of time so as to be useful in the printing processes of the present disclosure. The cross-linking agent can react with the hydroxyl groups or other moieties of the starch and/or PVOH to form the linkages between molecules. In an embodiment, cross-linking agents that can provide the desired degree of cross-linking at 180° C. or less, such as about 160° C. or 150°

C. or less, can be employed. In an embodiment, the cross-linking temperature ranges from about 80° C. to about 150° C. The time period for reaction may be in a range from about 0.1 second to about 10 minutes, depending on the temperature applied.

Examples of suitable cross-linking agents include tetraborate salts and hydrates thereof, such as sodium tetraborate decahydrate (borax); dialdehydes and hydrates thereof, such as glyoxal; ammonium zirconium carbonate; and cationic resins having a hydroxyl substituted quaternary amine group capable of reacting with hydroxyl groups of the waxy starch, such as polyamide-epichlorohydrin (“PAE”) resin, or a combination of any of the cross-linking agents described herein. An example of a commercially available cross-linking agent is BERSET® 2185, which is a glyoxal available from Bercen Inc. of Denham Springs, La. Another example of a commercially available cross-linking agent is POLYCUP 172, which is a polyamide-epichlorohydrin (“PAE”) resin available from Ashland Inc. of Covington, Kentucky. In an embodiment, the cross-linker is not cationic and/or does not contain an amino group.

Structural formulae and reactions with hydroxyl groups for PAE resin, borax and glyoxal are shown below, where n is the number of repeating units and R is any hydroxyl containing small molecule, oligomer or polymer (as understood in the art a small molecule is a low molecular weight compound, for example a compound having 1-20 monomer units, such as 1-4 monomer units):



R—OH <sup>HYDROXYL</sup>  
 $\downarrow$   
 $>100^\circ\text{C.}$



One, two, three or more of the cross-linkers can be employed together in the processes of the present disclosure. In an embodiment, both borax and glyoxal are employed together. One benefit of employing borax as a cross-linker is that the cross-linking can happen at a low temperature. For example, when the sacrificial coating solution is dried and the solid content of the PVOH and starch is increased to a desired level, the cross-linking can happen at room temperature with borax. However, the cross-linking can happen at around from 80° C. to around 90° C. with glyoxal cross-linker and around 100° C. to 120° C. for polyamide-epichlorohydrin (“PAE”) resin. All these cross-linkers are capable of cross-linking at room temperature when allowed to react over long periods of time, such as a few days, weeks or even months.

Examples of suitable polycarboxylic acid cross-linking agents include at least one compound selected from the group consisting of dicarboxylic acids, tricarboxylic acids, tetracarboxylic acids and water soluble polymeric carboxylic acids. In an embodiment, the compounds are dicarboxylic acids or tricarboxylic acids of formulae I or II:



where R<sup>1</sup> can be a saturated or unsaturated, linear, branched or cyclic, substituted or unsubstituted C<sub>1</sub> to C<sub>20</sub> carbon group optionally containing one or more heteroatoms. Examples of suitable R<sup>1</sup> groups include C<sub>1</sub> to C<sub>20</sub> alkanediyl, C<sub>1</sub> to C<sub>20</sub> alkenediyl, C<sub>1</sub> to C<sub>20</sub> bis alkylene ether, C<sub>1</sub> to C<sub>20</sub> cycloalky-

lene and  $C_1$  to  $C_{20}$  arenediyl; and  $R^2$  can be a saturated or unsaturated, linear, branched or cyclic, substituted or unsubstituted  $C_1$  to  $C_{20}$  carbon group, such as a  $C_1$  to  $C_{20}$  alkanyltriyl,  $C_1$  to  $C_{20}$  alkenetriyl,  $C_1$  to  $C_{20}$  cycloalkanetriyl or  $C_1$  to  $C_{20}$  arenetriyl. The  $R^1$  and  $R^2$  groups can optionally be substituted with one or more functional groups, such as hydroxyl groups, carbonyl group or amine groups.

Specific examples of suitable dicarboxylic acids of formula 1 include malonic acid, succinic acid, glutaric acid, adipic acid, pimelic acid, oleic acid dimer and sebacic acid. Specific examples of suitable tricarboxylic acids of formula 2 include pentane-1,3,5-tricarboxylic acid, benzene-1,3,5-tricarboxylic acid, isocitric acid, aconitic acid, propane-1,2,3-tricarboxylic acid, trimelic acid and citric acid. In an embodiment, the at least one tricarboxylic acid is citric acid. Polymeric carboxylic acids can also be employed. Specific examples of suitable water soluble polymeric carboxylic acids include poly(acrylic acid) and poly(methacrylic acid).

The amount of the cross-linking agent applied can be varied and depends on the type of cross-linking agent. Example amounts can range from about 2% to about 30% by weight, such as from about 2% to about 10% by weight, based on the total dry weight of the binders in the sacrificial coating. One, two, three or more of any of the above cross-linkers can be employed. For example, two or more of the cross-linkers can be combined and then applied to the wet sacrificial coating composition or the dry sacrificial coating in any manner described herein.

FIG. 1 illustrates a high-speed aqueous ink image producing machine or printer 10. As illustrated, the printer 10 is an indirect printer that forms an ink image on a surface of a blanket 21 mounted about an intermediate rotating member 12 and then transfers the ink image to media passing through a nip 18 formed between the blanket 21 and the transfix roller 19. The surface 14 of the blanket 21 is referred to as the image receiving surface of the blanket 21 and the rotating member 12 since the surface 14 receives a hydrophilic composition and the aqueous ink images that are transfixed to print media during a printing process. A print cycle is now described with reference to the printer 10. As used in this document, "print cycle" refers to the operations of a printer to prepare an imaging surface for printing, ejection of the ink onto the prepared surface, treatment of the ink on the imaging surface to stabilize and prepare the image for transfer to media, and transfer of the image from the imaging surface to the media.

The printer 10 includes a frame 11 that supports directly or indirectly operating subsystems and components, which are described below. The printer 10 includes an intermediate transfer member, which is illustrated as rotating imaging drum 12 in FIG. 1, but can also have other suitable configurations, such as a supported endless belt. The imaging drum 12 has an outer blanket 21 mounted about the circumference of the drum 12. The blanket moves in a direction 16 as the member 12 rotates. A transfix roller 19 rotatable in the direction 17 is loaded against the surface of blanket 21 to form a transfix nip 18, within which ink images formed on the surface of blanket 21 are transfixed onto a print medium 49. In some embodiments, a heater in the drum 12 (not shown) or in another location of the printer heats the image receiving surface 14 on the blanket 21 to a temperature in a range of, for example, approximately 50° C. to approximately 70° C. The elevated temperature promotes partial drying of the liquid carrier that is used to deposit the hydrophilic composition and of the water in the aqueous ink drops that are deposited on the image receiving surface 14.

The blanket is formed of a material having a relatively low surface energy to facilitate transfer of the ink image from the

surface of the blanket 21 to the print medium 49 in the nip 18. Such materials include polysiloxanes, fluoro-silicones, fluoropolymers such as VITON or TEFLON and the like. A surface maintenance unit (SMU) 92 removes residual ink left on the surface of the blanket 21 after the ink images are transferred to the print medium 49. The low energy surface of the blanket is not necessarily designed to aid in the formation of good quality ink images, at least because such surfaces do not spread ink drops as well as high energy surfaces.

10 In an embodiment more clearly depicted in FIG. 2, the SMU 92 includes a coating applicator, such as a donor roller 404, which is partially submerged in a reservoir 408 that holds the wet sacrificial coating compositions of the present disclosure. The donor roller 404 rotates in response to the movement of the image receiving surface 14 in the process direction. The donor roller 404 draws the liquid sacrificial coating composition from the reservoir 408 and deposits a layer of the composition on the image receiving surface 14. As described below, the sacrificial coating composition is deposited as a 15 uniform layer having any desired thickness. Examples include thicknesses ranging from about 0.1  $\mu$ m to about 10  $\mu$ m. The SMU 92 deposits the sacrificial coating composition on the image receiving surface 14. After a drying process, the dried sacrificial coating substantially covers the image receiving surface 14 before the printer ejects ink drops during a print process. In some illustrative embodiments, the donor roller 404 is an anilox roller or an elastomeric roller made of a material, such as rubber. The SMU 92 can be operatively connected to a controller 80, described in more detail below, to enable the controller to operate the donor roller, as well as a 20 metering blade and a cleaning blade, which may respectively function to deposit and distribute the coating material onto the surface of the blanket and to remove un-transferred ink and any sacrificial coating residue from the surface of the 25 blanket 21.

30 Referring back to FIG. 1, the printer 10 includes a dryer 96 that emits heat and optionally directs an air flow toward the wet sacrificial coating composition that is applied to the image receiving surface 14. The dryer 96 facilitates the 35 evaporation of at least a portion of the liquid carrier from the wet sacrificial coating composition to leave a dried layer on the image receiving surface 14 before the intermediate transfer member passes the printhead modules 34A-34D to receive the aqueous printed image.

45 The printer 10 can include an optical sensor 94A, also known as an image-on-drum ("IOD") sensor, which is configured to detect light reflected from the blanket surface 14 and the sacrificial coating applied to the blanket surface as the member 12 rotates past the sensor. The optical sensor 94A includes a linear array of individual optical detectors that are 50 arranged in the cross-process direction across the blanket 21. The optical sensor 94A generates digital image data corresponding to light that is reflected from the blanket surface 14 and the sacrificial coating. The optical sensor 94A generates 55 a series of rows of image data, which are referred to as "scanlines," as the intermediate transfer member 12 rotates the blanket 21 in the direction 16 past the optical sensor 94A. In one embodiment, each optical detector in the optical sensor 94A further comprises three sensing elements that are sensitive to wavelengths of light corresponding to red, green, and blue (RGB) reflected light colors. Alternatively, the optical sensor 94A includes illumination sources that shine red, green, and blue light or, in another embodiment, the sensor 94A has an illumination source that shines white light onto 60 the surface of blanket 21 and white light detectors are used. The optical sensor 94A shines complementary colors of light onto the image receiving surface to enable detection of dif- 65

ferent ink colors using the photodetectors. The image data generated by the optical sensor 94A can be analyzed by the controller 80 or other processor in the printer 10 to identify the thickness of the sacrificial coating on the blanket and the area coverage. The thickness and coverage can be identified from either specular or diffuse light reflection from the blanket surface and/or coating. Other optical sensors, such as 94B, 94C, and 94D, are similarly configured and can be located in different locations around the blanket 21 to identify and evaluate other parameters in the printing process, such as missing or inoperative inkjets and ink image formation prior to image drying (94B), ink image treatment for image transfer (94C), and the efficiency of the ink image transfer (94D). Alternatively, some embodiments can include an optical sensor to generate additional data that can be used for evaluation of the image quality on the media (94E).

The printer 10 includes an airflow management system 100, which generates and controls a flow of air through the print zone. The airflow management system 100 includes a printhead air supply 104 and a printhead air return 108. The printhead air supply 104 and return 108 are operatively connected to the controller 80 or some other processor in the printer 10 to enable the controller to manage the air flowing through the print zone. This regulation of the air flow can be through the print zone as a whole or about one or more printhead arrays. The regulation of the air flow helps prevent evaporated solvents and water in the ink from condensing on the printhead and helps attenuate heat in the print zone to reduce the likelihood that ink dries in the inkjets, which can clog the inkjets. The airflow management system 100 can also include sensors to detect humidity and temperature in the print zone to enable more precise control of the temperature, flow, and humidity of the air supply 104 and return 108 to ensure optimum conditions within the print zone. Controller 80 or some other processor in the printer 10 can also enable control of the system 100 with reference to ink coverage in an image area or even to time the operation of the system 100 so air only flows through the print zone when an image is not being printed.

The high-speed aqueous ink printer 10 also includes an aqueous ink supply and delivery subsystem 20 that has at least one source 22 of one color of aqueous ink. Since the illustrated printer 10 is a multicolor image producing machine, the ink delivery system 20 includes, for example, four (4) sources 22, 24, 26, 28, representing four (4) different colors CYMK (cyan, yellow, magenta, black) of aqueous inks. In the embodiment of FIG. 1, the printhead system 30 includes a printhead support 32, which provides support for a plurality of printhead modules, also known as print box units, 34A through 34D. Each printhead module 34A-34D effectively extends across the width of the blanket and ejects ink drops onto the surface 14 of the blanket 21. A printhead module can include a single printhead or a plurality of printheads configured in a staggered arrangement. Each printhead module is operatively connected to a frame (not shown) and aligned to eject the ink drops to form an ink image on the coating on the blanket surface 14. The printhead modules 34A-34D can include associated electronics, ink reservoirs, and ink conduits to supply ink to the one or more printheads. In the illustrated embodiment, conduits (not shown) operatively connect the sources 22, 24, 26, and 28 to the printhead modules 34A-34D to provide a supply of ink to the one or more printheads in the modules. As is generally familiar, each of the one or more printheads in a printhead module can eject a single color of ink. In other embodiments, the printheads can be configured to eject two or more colors of ink. For example, printheads in modules 34A and 34B can eject cyan and

magenta ink, while printheads in modules 34C and 34D can eject yellow and black ink. The printheads in the illustrated modules are arranged in two arrays that are offset, or staggered, with respect to one another to enable a continuous coverage of printing across the cross process width of the printing zone. Although the printer 10 includes four printhead modules 34A-34D, each of which has two arrays of printheads, alternative configurations include a different number of printhead modules or arrays within a module.

10 After the printed image on the blanket surface 14 exits the print zone, the image passes under an image dryer 130. The image dryer 130 includes a heater, such as a radiant infrared, radiant near infrared and/or a forced hot air convection heater 134, a dryer 136, which is illustrated as a heated air source 136, and air returns 138A and 138B. The infrared heater 134 applies infrared heat to the printed image on the surface 14 of the blanket 21 to evaporate water or solvent in the ink. The heated air source 136 directs heated air over the ink to supplement the evaporation of the water or solvent from the ink. In one embodiment, the dryer 136 is a heated air source with the same design as the dryer 96. While the dryer 96 is positioned along the process direction to dry the hydrophilic composition, the dryer 136 is positioned along the process direction 15 after the printhead modules 34A-34D to at least partially dry the aqueous ink on the image receiving surface 14. The air is then collected and evacuated by air returns 138A and 138B to reduce the interference of the air flow with other components in the printing area.

20 30 As further shown, the printer 10 includes a print medium supply and handling system 40 that stores, for example, one or more stacks of paper print mediums of various sizes. The print medium supply and handling system 40, for example, includes sheet or substrate supply sources 42, 44, 46, and 48.

25 35 In the embodiment of printer 10, the supply source 48 is a high capacity paper supply or feeder for storing and supplying image receiving substrates in the form of cut print mediums 49, for example. The print medium supply and handling system 40 also includes a substrate handling and transport system 50 that has a media pre-conditioner assembly 52 and a media post-conditioner assembly 54. The printer 10 includes an optional fusing device 60 to apply additional heat and pressure to the print medium after the print medium passes through the transfix nip 18. In the embodiment of FIG. 1, the printer 10 includes an original document feeder 70 that has a 40 document holding tray 72, document sheet feeding and retrieval devices 74, and a document exposure and scanning system 76.

30 45 50 Operation and control of the various subsystems, components and functions of the machine or printer 10 are performed with the aid of a controller or electronic subsystem (ESS) 80. The ESS or controller 80 is operably connected to, for example, the intermediate transfer member 12, the printhead modules 34A-34D (and thus the printheads), the substrate supply and handling system 40, the substrate handling and transport system 50, and, in some embodiments, the one or more optical sensors 94A-94E. The ESS or controller 80, for example, is a self-contained, dedicated mini-computer having a central processor unit (CPU) 82 with electronic storage 84, and a display or user interface (UI) 86. The ESS or controller 80, for example, includes a sensor input and control circuit 88 as well as a pixel placement and control circuit 89. In addition, the CPU 82 reads, captures, prepares and manages the image data flow between image input sources, such as the scanning system 76, or an online or a work station connection 90, and the printhead modules 34A-34D. As such, the ESS or controller 80 is the main multi-tasking processor

for operating and controlling all of the other machine subsystems and functions, including the printing process discussed below.

The controller 80 can be implemented with general or specialized programmable processors that execute programmed instructions. The instructions and data required to perform the programmed functions can be stored in memory associated with the processors or controllers. The processors, their memories, and interface circuitry configure the controllers to perform the operations described below. These components can be provided on a printed circuit card or provided as a circuit in an application specific integrated circuit (ASIC). Each of the circuits can be implemented with a separate processor or multiple circuits can be implemented on the same processor. Alternatively, the circuits can be implemented with discrete components or circuits provided in very large scale integrated (VLSI) circuits. Also, the circuits described herein can be implemented with a combination of processors, ASICs, discrete components, or VLSI circuits.

Although the printer 10 in FIG. 1 is described as having a blanket 21 mounted about an intermediate rotating member 12, other configurations of an image receiving surface can be used. For example, the intermediate rotating member can have a surface integrated into its circumference that enables an aqueous ink image to be formed on the surface. Alternatively, a blanket is configured as an endless rotating belt for formation of an aqueous image. Other variations of these structures can be configured for this purpose. As used in this document, the term "intermediate imaging surface" includes these various configurations.

Once an image or images have been formed on the blanket and coating under control of the controller 80, the illustrated inkjet printer 10 operates components within the printer to perform a process for transferring and fixing the image or images from the blanket surface 14 to media. In the printer 10, the controller 80 operates actuators to drive one or more of the rollers 64 in the media transport system 50 to move the print medium 49 in the process direction P to a position adjacent the transfix roller 19 and then through the transfix nip 18 between the transfix roller 19 and the blanket 21. The transfix roller 19 applies pressure against the back side of the print medium 49 in order to press the front side of the print medium 49 against the blanket 21. Although the transfix roller 19 can also be heated, in the exemplary embodiment of FIG. 1 the transfix roller 19 is unheated. Instead, the pre-heater assembly 52 for the print medium 49 is provided in the media path leading to the nip. The pre-conditioner assembly 52 conditions the print medium 49 to a predetermined temperature that aids in the transferring of the image to the media, thus simplifying the design of the transfix roller. The pressure produced by the transfix roller 19 on the back side of the heated print medium 49 facilitates the transfixing (transfer and fusing) of the image from the intermediate transfer member 12 onto the print medium 49. The rotation or rolling of both the intermediate transfer member 12 and transfix roller 19 not only transfixes the images onto the print medium 49, but also assists in transporting the print medium 49 through the nip. The intermediate transfer member 12 continues to rotate to enable the printing process to be repeated.

After the intermediate transfer member 12 moves through the transfix nip 18, the image receiving surface passes a cleaning unit that removes residual portions of the sacrificial coating and small amounts of residual ink from the image receiving surface 14. In the printer 10, the cleaning unit is embodied as a cleaning blade 95 that engages the image receiving surface 14. The blade 95 is formed from a material that wipes the image receiving surface 14 without causing

damage to the blanket 21. For example, the cleaning blade 95 is formed from a flexible polymer material in the printer 10. As depicted below in FIG. 1, another embodiment has a cleaning unit that includes a roller or other member that applies a mixture of water and detergent to remove residual materials from the image receiving surface 14 after the intermediate transfer member moves through the transfix nip 18. As used herein, the term "detergent" or cleaning agent refers to any surfactant, solvent, or other chemical compound that is suitable for removing any sacrificial coating and any residual ink that may remain on the image receiving surface from the image receiving surface. One example of a suitable detergent is sodium stearate, which is a compound commonly used in soap. Another example is IPA, which is common solvent that is very effective to remove ink residues from the image receiving surface. In an embodiment, no residue of the sacrificial coating layer remains on the ITM after transferring the ink and sacrificial layer, in which case cleaning of the ITM to remove residual sacrificial coating may not be an issue.

FIG. 3 depicts a process 700 for operating an aqueous indirect inkjet printer using a sacrificial coating composition, as described herein, to form a dried coating on an image receiving surface of an intermediate transfer member prior to ejecting liquid ink drops onto the dried layer. In the discussion below, a reference to the process 700 performing an action or function refers to a controller, such as the controller 80 in the printer 10, executing stored programmed instructions to perform the action or function in conjunction with other components of the printer. The process 700 is described in conjunction with FIG. 1 showing the printer 10, and FIG. 4A—FIG. 4E showing the blanket and coatings, for illustrative purposes. The sacrificial coatings and processes of employing these coatings are not limited to use with printer 10, but can potentially be employed with any inkjet printer comprising an intermediate transfer member, as would be readily understood by one of ordinary skill in the art.

Process 700 begins as the printer applies a sacrificial layer of a wet coating composition with a liquid carrier to the image receiving surface of the intermediate transfer member (block 704). In the printer 10, the drum 12 and blanket 21 move in the process direction along the indicated circular direction 16 during the process 700 to receive the sacrificial coating composition.

In an embodiment, the liquid carrier is water or another liquid, such as alcohol or any of the other liquid carriers described herein for use in the wet coating composition, which partially evaporates from the image receiving surface and leaves a dried layer on the image receiving surface. In FIG. 4A, the surface of the intermediate transfer member 504 is covered with the sacrificial coating composition 508. The SMU 92 deposits the sacrificial coating composition on the image receiving surface 14 of the blanket 21 to form a uniform hydrophilic coating. A greater coating thickness of the sacrificial coating composition enables formation of a uniform layer that completely covers the image receiving surface, but the increased volume of liquid carrier in the thicker coating requires additional drying time or larger dryers to remove the liquid carrier to form a dried layer. Thinner coatings of the sacrificial coating composition require the removal of a smaller volume of the liquid carrier to form the dried layer, but if the sacrificial coating is too thin, then the coating may not fully cover the image receiving surface. In certain embodiments the sacrificial coating composition with the liquid carrier is applied at a thickness of between approximately 1  $\mu\text{m}$  and 10  $\mu\text{m}$ .

Process 700 continues as a dryer in the printer dries the sacrificial coating composition to remove at least a portion of

the liquid carrier and to form a dried layer on the image receiving surface (block 708). In the printer 10 the dryer 96 applies radiant heat and optionally includes a fan to circulate air onto the image receiving surface of the drum 12. FIG. 4B depicts the dried layer 512. The dryer 96 removes a portion of the liquid carrier, which decreases the thickness of the layer of dried layer that is formed on the image receiving surface. In the printer 10 the thickness of the dried layer 512 can be any suitable desired thickness. Example thicknesses range from about 0.1  $\mu\text{m}$  to about 3  $\mu\text{m}$  in different embodiments, and in certain specific embodiments from about 0.1 to about 0.5  $\mu\text{m}$ .

The dried sacrificial coating 512 is also referred to as a "skin" layer. The dried sacrificial coating 512 has a uniform thickness that covers substantially all of the portion of the image receiving surface that receives aqueous ink during a printing process. As described above, while the sacrificial coating with the liquid carrier includes solutions, suspension, or dispersion of the sacrificial coating material in a liquid carrier, the dried sacrificial coating 512 covers the image receiving surface of intermediate transfer member 504. The dried sacrificial coating 512 has a comparatively high level of adhesion to the image receiving surface of intermediate transfer member 504, and a comparatively low level of adhesion to a print medium that contacts the dried layer 512. As described in more detail below, when aqueous ink drops are ejected onto portions of the dried layer 512, a portion of the water and other solvents in the aqueous ink permeates the dried layer 512.

Process 700 continues as the image receiving surface with the hydrophilic skin layer moves past one or more printheads that eject aqueous ink drops onto the dried layer and the image receiving surface to form a latent aqueous printed image (block 712). The printhead modules 34A-34D in the printer 10 eject ink drops in the CMYK colors to form the printed image.

The sacrificial coating 512 is substantially impermeable to the colorants in the ink 524, and the colorants remain on the surface of the dried layer 512 where the aqueous ink spreads. The spread of the liquid ink enables neighboring aqueous ink drops to merge together on the image receiving surface instead of beading into individual droplets as occurs in traditional low-surface energy image receiving surfaces.

Referring again to FIG. 3, the process 700 continues with a partial drying process of the aqueous ink on the intermediate transfer member (block 716). The drying process removes a portion of the water from the aqueous ink and the sacrificial coating, also referred to as the skin layer, on the intermediate transfer member so that the amount of water that is transferred to a print medium in the printer does not produce cockling or other deformations of the print medium. In the printer 10, the heated air source 136 directs heated air toward the image receiving surface 14 to dry the printed aqueous ink image. In some embodiments, the intermediate transfer member and blanket are heated to an elevated temperature to promote evaporation of liquid from the ink. For example, in the printer 10, the imaging drum 12 and blanket 21 are heated to a temperature of 50° C. to 70° C. to enable partial drying of the ink on the dried sacrificial layer during the printing process. As depicted in FIG. 4D, the drying process forms a partially dried aqueous ink 532 that retains a reduced amount of water compared to the freshly printed aqueous ink image of FIG. 4C.

The drying process increases the viscosity of the aqueous ink, which changes the consistency of the aqueous ink from a low-viscosity liquid to a higher viscosity tacky material. The drying process also reduces the thickness of the ink 532. In an embodiment, the drying process removes sufficient water so

that the ink contains less than 20% water by weight, such as less than 5% water, or even less than 2% water, by weight of the partially dried ink (the ink after drying but before transfer to the print medium).

5 Process 700 continues as the printer transfixes the latent aqueous ink image from the image receiving surface to a print medium, such as a sheet of paper (block 720). In the printer 10, the image receiving surface 14 of the drum 12 engages the transfix roller 19 to form a nip 18. A print medium, such as a 10 sheet of paper, moves through the nip between the drum 12 and the transfix roller 19. The pressure in the nip transfers the aqueous ink image and a portion of the dried sacrificial layer to the print medium. After passing through the transfix nip 18, the print medium carries the printed aqueous ink image. As 15 depicted in FIG. 4E, a print medium 536 carries a printed aqueous ink image 532 with the sacrificial coating 512 covering the ink image 532 on the surface of the print medium 536. The sacrificial coating 512 provides protection to the aqueous ink image from scratches or other physical damage 20 while the aqueous ink image 532 dries on the print medium 536.

During process 700, the printer cleans any residual portions 25 of the sacrificial coating 512 that may remain on the image receiving surface after the transfixing operation (block 724). In one embodiment, a cleaning system uses, for example, a combination of water and a detergent with 30 mechanical agitation on the image receiving surface to remove the residual portions of the sacrificial coating 512 from the surface of the drum 12. In the printer 10, a cleaning blade 95, which can be used in conjunction with water, engages the blanket 21 to remove any residual sacrificial coating 512 from the image receiving surface 14. The cleaning blade 95 is, for example, a polymer blade that wipes 35 residual portions of the sacrificial coating 512 from the blanket 21.

During a printing operation, process 700 returns to the 40 processing described above with reference to block 704 to apply the hydrophilic composition to the image receiving surface, print additional aqueous ink images, and transfix the aqueous ink images to print media for additional printed 45 pages in the print process. The illustrative embodiment of the printer 10 operates in a "single pass" mode that forms the dried layer, prints the aqueous ink image and transfixes the aqueous ink image to a print medium in a single rotation or circuit of the intermediate transfer member. In alternative 50 embodiments, an inkjet employs a multi-pass configuration where the image receiving surface completes two or more rotations or circuits to form the dried layer and receive the aqueous ink image prior to transfixing the printed image to the print medium.

In some embodiments of the process 700, the printer forms 55 printed images using a single layer of ink such as the ink 524 that is depicted in FIG. 4C. In the printer 10, however, the multiple printhead modules enable the printer to form printed images with multiple colors of ink. In other embodiments of the process 700, the printer forms images using multiple ink colors. In some regions of the printed image, multiple colors of ink may overlap in the same area on the image receiving surface, forming multiple ink layers on the hydrophilic composition layer. The method steps in FIG. 3 can be applied to 60 the multiple ink layer circumstance with similar results.

Referring to 730 of FIG. 3, the at least one cross-linking 65 agent can be applied to cross-link the sacrificial coating at any suitable time during the process 700. In an embodiment, the cross-linking agent can be applied to the intermediate transfer member at point 732 in the process, prior to depositing the wet sacrificial coating composition. In this case, the cross-

19

linking agent is applied directly onto the intermediate transfer member, such as by spray coating, roll coating or any other suitable method. The cross linking agent then comes into contact with the sacrificial coating composition at 704 when the sacrificial coating composition is subsequently applied to the intermediate transfer member.

In another embodiment, the cross-linking agent is applied directly to the wet sacrificial coating composition 508 (FIG. 4A) at point 734 in the process. Alternatively, the cross-linking agent can be applied after drying, e.g., to the dried sacrificial coating 512 (FIG. 4B), such as prior to the ink being ejected (e.g., at point 736), or at any time after the ink is ejected onto the sacrificial coating (e.g., points 738 or 740). In yet another embodiment, the cross-linking agent can be combined with the ink and then ejected with the ink composition onto the dry sacrificial coating. In processes where multiple colors of ink are employed, the cross-linking agent can be applied in between different colors, such as after the ejecting of a first color onto the dry sacrificial coating and prior to the ejecting of a second color onto the dry sacrificial coating.

Alternatively, the cross-linking agent can be applied to the dry sacrificial coating after transfer of the sacrificial coating onto the print medium 536, such as at point 742 in the process. This can occur before or after any optional final drying of the ink and/or sacrificial coating that is carried out after transfer to the print medium 536. For any of the processes disclosed herein, additional drying of the cross-linking agent may optionally be performed immediately after application of the cross-linking agent.

The cross linking agent can be applied using any suitable technique. Suitable coating techniques can include any contact coating technique, e.g., roll coating, slot-die coating or dip coating, and any non-contact coating techniques, e.g., spray coating. A combination of contact and non-contact coating techniques can also be used. One example of a roll coating technique involves the use of an anilox roller, such as shown in FIG. 2, which can be used to apply the cross-linking agent onto either the intermediate transfer member or the sacrificial coating.

## EXAMPLES

### Example 1

#### Sacrificial Coating Compositions

Various example sacrificial coating compositions are shown in Tables 1A and 1B. All percentages in the examples below are weight percentages based on the total weight of the composition, unless otherwise stated.

TABLE 1A

| Dry Components                          | Sacrificial coating formulations for air brush: |              |              |
|-----------------------------------------|-------------------------------------------------|--------------|--------------|
|                                         | Control Sample 1-1                              | Example 1-1A | Example 1-1B |
| Caliber 180 Starch (waxy maize starch)* | 1.6                                             | 1.6          | 1.6          |
| Selvol PVOH 825**                       | 0.4                                             | 0.4          | 0.4          |
| Glycerol                                | 6.7                                             | 6.7          | 6.7          |
| Borax                                   | 0                                               | 0.65         | 0.65         |
| Berset2185 (Glyoxal)                    |                                                 |              | 0.3          |
| SLS                                     | 0.1                                             | 0.1          | 0.1          |
| Water                                   | 91.2                                            | 90.55        | 90.25        |
| Total                                   | 100                                             | 100          | 100          |

20

TABLE 1B

| Sacrificial coating with PAE resin for air brush |                    |              |
|--------------------------------------------------|--------------------|--------------|
| Dry formulation                                  | Control Sample 1-2 | Example 1-2A |
| Starch Caliber 180*                              | 1.6                | 1.6          |
| PVOH 825**                                       | 0.4                | 0.4          |
| PAE                                              |                    | 0.4          |
| Glycerol                                         | 6.7                | 6.7          |
| SLS                                              | 0.1                | 0.1          |
| Water                                            | 91.2               | 91.2         |
| Total: 100                                       | 100                | 100          |

\*Starch Caliber 180 was cooked at 10% solid, 93° C. for 15 minutes.

\*\*PVOH 825 was cooked at 10% at 93° C. for 60 minutes

### Example 2

#### Air Brush Sample Preparation

The samples of Example 1 were implemented using a surrogate testing method. Rather than printing the skin and ink in two separate steps as in the above described methods of the present disclosure, the skin and ink formulations were combined and applied as one layer, and then dried. It has been demonstrated that when the skin and ink are applied separately, they do not form two distinct layers as might be expected, but merge into a single mixed layer, as is the case when the two liquids are combined and printed in a single pass. Good correlation for certain testing purposes has been observed between this surrogate method and the two step process generally used for indirect print testing, as described herein.

Air brush samples were prepared as follows:

- Solution preparation: Each of the sacrificial coating solutions of Control Sample 1-1 and Examples 1-1A and 1-1B were mixed with an experimental aqueous black ink at a premix ink to skin ratio of 1:1. The sacrificial coating solutions of Control Sample 1-2 and Example 1-1A were mixed with the experimental aqueous ink in three separate solutions at a premix ink to skin ratio of 1:1, a premix ink to skin ratio of 1:3 and premix ink to skin ratio of 1:9. Thus, the sacrificial skin loading was equal to or higher than the ink in each case. It has been found that the higher the sacrificial skin loading is, the worse will be the water fastness.
- Air brush process: In order to generate a rectangular air brushed image, an image template was created by cutting out a 2.5 cm x 15 cm rectangular slit from a piece of stainless steel metal. The template was put on top of the paper before air brushing so the rectangular image can be generated. The solutions from step a) were sprayed on the paper using an Iwata HP-C Plus Japan MH air brush until the image was opaque and uniform, with optical density around 1.5.
- Drying process: The air brushed sheet was put into an oven and dried at 92° C. at a fan speed of 700 rpm air flow for 2 minutes.
- Sheet condition: The air brushed sheet was conditioned at 23° C. and at a relative humidity of about 50% for at least one hour.

### Example 3

#### Sacrificial Coating Compositions for Aqueous Ink Indirect Print Testing

Various sacrificial coating compositions (shown as Examples 3-1A to 3-3B) were made for Aqueous Ink Indirect

## 21

Print Testing. The ingredients and amounts are shown in Tables 2 and 3. All percentages in Tables 2 and 3 are weight percentages based on the total weight of the composition.

TABLE 2

| Dry formulation    | Control    |        | Example    |        |
|--------------------|------------|--------|------------|--------|
|                    | Sample 3-1 | 3-1A   | Sample 3-2 | 3-2A   |
| Starch Caliber 180 | 1.6        | 1.6    | 1.28       | 1.28   |
| PVOH 825           | 0.4        | 0.4    |            |        |
| PVOH 350           |            |        | 0.32       | 0.32   |
| Glycerol           | 6.7        | 6.7    | 5.34       | 5.34   |
| 2-Pyrrolidinone    |            |        | 1.36       | 1.36   |
| SLS                | 0.1        | 0.1    | 0.1        | 0.1    |
| Borax              |            | 0.325  |            | 0.325  |
| Water              | 91.2       | 90.875 | 91.6       | 91.275 |
| Total: 100         | 100        | 100    | 100        | 100    |

TABLE 3

| Dry formulation    | Additional Sacrificial coating formulations for Indirect Print Testing |              |              |
|--------------------|------------------------------------------------------------------------|--------------|--------------|
|                    | Control Sample 3-3                                                     | Example 3-3A | Example 3-3B |
| Starch Caliber 180 | 1.6                                                                    | 1.12         | 1.2          |
| PVOH 825           | 0.4                                                                    |              |              |
| PVOH 350           |                                                                        | 0.24         | 0.2          |
| Glycerol           | 6.7                                                                    | 6.7          | 6.03         |
| 2-Pyrrolidinone    |                                                                        |              | 0.67         |
| SLS                | 0.1                                                                    | 0.1          | 0.1          |
| Borax              |                                                                        | 0.4          | 0.5          |
| Water              | 91.2                                                                   | 91.44        | 91.3         |
| Total: 100         | 100                                                                    | 100          | 100          |

## Example 4

## Indirect Print Testing Procedure

The print testing was carried out using a printing fixture, such as is generically illustrated in FIG. 1. The sacrificial coating, sometimes referred to herein as the “skin”, was applied on the blanket of the fixture in a solution form and then dried. This formed a strong and robust film layer with a thickness of from about 0.1 to about 0.5 microns on top of the blanket. The ink was then jetted on top of the skin and semi-dried before the entire layer of ink and skin was transferred on to the substrate. Various process conditions were varied to test the system latitude and images were examined to evaluate the system performance. Compared to formulations without cross-linker, the new formulations showed similar performance in terms of wet image quality and ink transfer.

## Example 5

## Water Fastness Test Procedure

Water fastness smear testing was conducted using Taber linear abraser—Model 5700 on both the airbrush samples and the print testing samples discussed above. Before the testing, a piece of cloth (TIC Crockmeter Squares 2"×2"-product code: M238CT) was attached to the bottom of the shaft and held in place using a clip. Then a drop of water having a volume of about 0.10-0.12 ml was put on the image area using a needle. After 1 minute had passed, the shaft (weight 417.7 g)

## 22

was lowered so that it rested against the ink surface. Immediately, the start switch was flipped on the linear abraser and stopped after it had completed half a cycle, thereby forming smear samples as shown in FIG. 5B.

## 5 Smear OD Ratio:

The optical density was measured using X-Rite device on the original sample area prior to water fastness testing, and again measured on the smear area after water fastness testing. The optical density (“OD”) ratio was calculated by smear OD/Original OD\*100.

10 The smear OD ratio results for the airbrush samples of Table 1A are shown in FIG. 5A. As is apparent from the data, the formulations of Examples 1-1A and 1-1B with cross-linking agent resulted in a larger percent smear ratio, indicating an improvement in that less ink was removed from these samples than was removed from the Control sample 1 formulation without cross-linkers. A visual inspection of the samples after the water fastness testing was performed showed smudging was apparent for the Control sample 1. 15 Considerably less smudging occurred for the Example 1A formulation with the Borax cross-linking agent, while no noticeable smudging was apparent from the Example 1B composition with both Borax and Glyoxal cross-linking agents.

20 25 Smear OD ratio results for the airbrush samples of Table 1B mixed at the various ink to skin ratios as described in Example 2 were also obtained. Results are shown in FIG. 5B. Significant improvement in water fastness was exhibited with polyamide-epichlorohydrin (“PAE”) at all ink:skin ratios 30 when compared to the same formulations using PVOH instead of PAE. The lower the proportion of ink, the worse the water fastness results were. Almost no ink transferred at a 50:50 ratio of ink:skin using the skin formulation of Example 1-2A.

35 The smear OD ratio data for the examples shown in Table 2 is shown in FIG. 6, for the skin formulations printed with black ink, and in FIG. 7, for the skin formulations printed with magenta ink. The smear OD ratio data for the examples shown in Table 3 is shown in FIG. 8, for the skin formulations printed with black ink, and FIG. 9, for the skin formulations printed with magenta ink. Skin formulations with cross-linking agent consistently showed improved water fastness compared to those without.

## Example 6

45 50 55 Sacrificial coating solutions of Example 6-1 and Example 6-2 were made with different PAE loadings, as shown in Tables 4-1 and 4-2. The sacrificial coating solutions were mixed with the experimental aqueous black ink at a premix ink to skin ratio of 1:3. Water fastness testing was conducted on formulations with the different PAE loadings to identify the loadings that provide the best water fastness performance. The water fastness screening test procedure was the same as described above in Example 5. The water fastness results are shown in FIGS. 10A and 10B. The values in Tables 4-1 and 4-2 are in weight percent based on the total weight of the composition.

## TABLE 4-1

| Components | Control Sample 6-1 | Example 6-1A | Example 6-1B | Example 6-1C | Example 6-1D |
|------------|--------------------|--------------|--------------|--------------|--------------|
| Starch     | 1.6                | 1.6          | 1.6          | 1.6          | 1.6          |
| PVOH 350   | 0.4                | 0.3          | 0.2          | 0.1          | 0            |

TABLE 4-1-continued

| Components       | Control Sample 6-1 | Example 6-1A | Example 6-1B | Example 6-1C | Example 6-1D |
|------------------|--------------------|--------------|--------------|--------------|--------------|
| Polycup172 (PAE) |                    | 0.1          | 0.2          | 0.3          | 0.4          |
| Glycerol         | 6.7                | 6.7          | 6.7          | 6.7          | 6.7          |
| SLS              | 0.1                | 0.1          | 0.1          | 0.1          | 0.1          |
| Water            | 91.2               | 91.2         | 91.2         | 91.2         | 91.2         |
| Total            | 100                | 100          | 100          | 100          | 100          |

TABLE 4-2

| Components        | Example 6-2A | Example 6-2B | Example 6-2C | Example 6-2D | Example 6-2E | Example 6-2F |
|-------------------|--------------|--------------|--------------|--------------|--------------|--------------|
| Starch            | 1.9          | 1.8          | 1.7          | 1.6          | 1.5          | 1.4          |
| Poly-cup172 (PAE) | 0.1          | 0.2          | 0.3          | 0.4          | 0.5          | 0.6          |
| Glycerol          | 6.7          | 6.7          | 6.7          | 6.7          | 6.7          | 6.7          |
| SLS               | 0.1          | 0.1          | 0.1          | 0.1          | 0.1          | 0.1          |
| Water             | 91.2         | 91.2         | 91.2         | 91.2         | 91.2         | 91.2         |
| Total             | 100          | 100          | 100          | 100          | 100          | 100          |

Water fastness data for the formulations of Table 4-1 is shown in FIG. 10A. Water fastness data for the formulations of Table 4-2 is shown in FIG. 10B. As shown in FIG. 10A, from varying the PVOH:PAE ratio while keeping the starch loading and total binder the same, it was found that 100% PVOH replacement with PAE was the best for water fastness. As shown in FIG. 10B, varying the starch:PAE ratio with no PVOH, an about 0.4% to about 0.5% by weight PAE loading was found to produce good results.

The above example sacrificial coating formulations were shown to have improved print performance based on image quality and water fastness, as confirmed by the marking tests and print testing above. By loading borax, glyoxal or mixtures of glyoxal and borax as cross-linkers, the water fastness was significantly improved.

### Example 7

#### Sacrificial Coating Composition

A drop of 5% by weight solution of citric acid was added to a half tone print having a sacrificial coating positioned thereon (similarly as made in the process described above, an example of which print is illustrated in FIG. 4E). The citric acid was dried at 120° C. The area of the print treated with citric acid showed significantly improved water fastness compared to non-treated areas, areas that had been treated with a drop of water and dried, and areas that had been treated with a drop of 5% by weight Borax solution and dried.

Notwithstanding that the numerical ranges and parameters setting forth the broad scope of the disclosure are approximations, the numerical values set forth in the specific examples are reported as precisely as possible. Any numerical value, however, inherently contains certain errors necessarily resulting from the standard deviation found in their respective testing measurements. Moreover, all ranges disclosed herein are to be understood to encompass any and all sub-ranges subsumed therein.

While the present teachings have been illustrated with respect to one or more implementations, alterations and/or

modifications can be made to the illustrated examples without departing from the spirit and scope of the appended claims. In addition, while a particular feature of the present teachings may have been disclosed with respect to only one of several implementations, such feature may be combined with one or more other features of the other implementations as may be desired and advantageous for any given or particular function. Furthermore, to the extent that the terms "including," "includes," "having," "has," "with," or variants thereof are used in either the detailed description and the claims, such terms are intended to be inclusive in a manner similar to the term "comprising." Further, in the discussion and claims herein, the term "about" indicates that the value listed may be somewhat altered, as long as the alteration does not result in nonconformance of the process or structure to the illustrated embodiment. Finally, "exemplary" indicates the description is used as an example, rather than implying that it is an ideal.

It will be appreciated that variants of the above-disclosed and other features and functions, or alternatives thereof, may be combined into many other different systems or applications. Various presently unforeseen or unanticipated alternatives, modifications, variations, or improvements therein may be subsequently made by those skilled in the art which are also intended to be encompassed by the following claims.

What is claimed is:

1. An indirect printing process comprising:  
providing an inkjet printing apparatus comprising an intermediate transfer member;  
depositing a wet sacrificial coating composition onto the intermediate transfer member, the wet sacrificial coating composition made from ingredients comprising:  
a waxy starch;  
at least one hygroscopic material;  
at least one surfactant; and  
a liquid carrier;  
drying the wet sacrificial coating composition to form a dry sacrificial coating;  
ejecting droplets of ink in an imagewise pattern onto the dry sacrificial coating;  
at least partially drying the ink to form a substantially dry ink pattern;  
transferring both the substantially dry ink pattern and the sacrificial coating from the intermediate transfer member to a final substrate; and  
applying at least one cross-linking agent to cross-link the sacrificial coating, wherein the cross-linking agent is applied to at least one of: a) the intermediate transfer member prior to depositing the wet sacrificial coating composition, b) the wet sacrificial coating composition after depositing the wet sacrificial coating composition onto the intermediate transfer member, c) the dry sacrificial coating on the intermediate transfer member, or d) the dry sacrificial coating on the final substrate.

2. The process of claim 1, wherein the cross-linking agent is applied to the dry sacrificial coating on the intermediate transfer member.

3. The process of claim 2, wherein the cross-linking agent is combined with the ink and ejected onto the dry sacrificial coating.

4. The process of claim 2, wherein the cross-linking agent is applied onto the dry sacrificial coating prior to the droplets of ink.

5. The process of claim 2, further comprising ejecting multiple colors of ink, wherein the cross-linking agent is applied after the ejecting of a first color onto the dry sacrificial coating and prior to the ejecting of a second color onto the dry sacrificial coating.

## 25

6. The process of claim 2, wherein the cross-linking agent is applied onto the dry sacrificial coating after the imagewise pattern of ink is formed onto the dry sacrificial coating.

7. The process of claim 1, wherein the cross-linking agent is applied by a coating technique selected from the group consisting of spray coating, roll coating, slot-die coating and dip coating.

8. The process of claim 1, wherein the cross-linking agent is a polycarboxylic acid.

9. The process of claim 8, wherein the polycarboxylic acid is selected from the group consisting of dicarboxylic acids and tricarboxylic acids.

10. The process of claim 1, wherein the cross-linking agent is selected from the group consisting of tetraborate salts and hydrates thereof, dialdehydes and hydrates thereof, ammonium zirconium carbonate, a cationic resin having a hydroxyl substituted quaternary amine group and combinations thereof.

11. The process of claim 1, wherein the cross-linking agent is selected from the group consisting of sodium tetraborate decahydrate, glyoxal, ammonium zirconium carbonate, polyamide-epichlorohydrin resin or a combination thereof.

12. The process of claim 1, wherein the waxy starch comprises at least one starch selected from the group consisting of a waxy maize starch, a waxy rice starch, a waxy cassava starch, a waxy potato starch, a waxy wheat starch and a waxy barley starch.

13. The process of claim 1, wherein the sacrificial coating composition further comprising at least one polymer selected

## 26

from the group consisting of i) polyvinyl alcohol and ii) a copolymer of vinyl alcohol and alkene monomers.

14. The process of claim 1, wherein the at least one polycarboxylic acid is citric acid.

15. The process of claim 1, wherein the at least one polycarboxylic acid is a water soluble polymeric carboxylic acid.

16. The process of claim 1, wherein the sacrificial coating composition further comprising at least one polymer selected from the group consisting of i) polyvinyl alcohol and ii) a copolymer of vinyl alcohol and alkene monomers.

17. The process of claim 1, wherein the at least one hydroscopic material is selected from the group consisting of glycerol, sorbitol, glycols and mixtures thereof.

18. The process of claim 1, wherein the liquid carrier further comprises at least one solvent selected from the group consisting of isopropanol, methyl ethyl ketone, 2-pyrrolidinone, terpineol, dimethylsulfoxide, N-methylpyrrolidone, 1,3-dimethyl-2-imidazolidinone, 1,3-dimethyl-3,4,5,6-tetrahydro-2 pyrimidinone or dimethylpropylene urea and the mixtures thereof.

19. The process of claim 1, wherein the at least one surfactant is selected from the group consisting of an anionic surfactant, a non-ionic surfactant and a combination of both an anionic surfactant and a non-ionic surfactant.

20. The process of claim 1, wherein the at least one surfactant is a non-ionic surfactant having an HLB value ranging from about 4 to about 14.

\* \* \* \* \*